

## UNITED STATES PATENT OFFICE

2,041,866

## MULTIPLE ALLOYS

Georg Schichtel, Radenthein, Austria, assignor  
to American Magnesium Metals Corporation,  
Pittsburgh, Pa., a corporation of Delaware

No Drawing. Original application November 18,  
1932, Serial No. 643,297. Divided and this ap-  
plication June 4, 1935, Serial No. 24,979. In  
Austria February 19, 1932

5 Claims. (Cl. 75—168)

This application is a division of my prior ap-  
plication Serial No. 643,297, filed November 18,  
1932.

The present improved alloy is one in which  
5 magnesium is the predominant element, the pri-  
mary object being to develop an alloy that will  
possess the characteristic low specific gravity  
which is obtained by the use of magnesium in ex-  
cess of 80 per cent while such alloy will be char-  
acterized by higher resistance to corrosion and  
10 at the same time will have a higher strength than  
the known alloys of this kind.

The known alloys in use containing generally  
more than 85% magnesium and as principal ad-  
15 ditional ingredient aluminum or zinc or both of  
these ingredients, other constituents being pres-  
ent in relatively small amounts, do not exhibit a  
sufficient resistance to corrosion by water or even  
20 by damp air, and cannot be used at all when in  
continuous contact with sea-water. Various at-  
tempts have been made to render the surfaces  
of these metals more resistant by applying coat-  
ings, but such attempts failed since corrosion  
25 often takes place to an increased extent when  
the superficial protective layer is damaged.

The object of the invention is attained by the  
addition of further additional metals to the al-  
loys, namely antimony or bismuth or both of these  
metals amounting in general to not less than  
30 0.05% and not more than 2% of the total.

The most diverse alloys of the kind referred  
to containing antimony or bismuth have proved  
35 distinctly superior, when exposed to the action  
of a 3% solution of common salt, to alloys of the  
same kind which do not contain antimony or  
bismuth; whilst the alloys containing antimony  
40 or bismuth showed an almost unaltered surface,  
the samples devoid of antimony or bismuth were  
strongly corroded on carrying out the compara-  
tive tests.

In general the lower limit of efficiency is given  
by additions of 0.05%, and it is preferable not  
to exceed the upper limit of 2%.

From their position in the electrochemical se-  
ries antimony and bismuth are more valuable  
45 than magnesium, and moreover do not form a  
solid solution with the latter; the assumption  
therefore would rather have been that the ad-  
dition of these metals to the known alloys of mag-  
50 neesium would involve decreasing their resistance  
to corrosion.

The magnesium-base alloys developed by the  
present invention show also a considerable in-  
crease in strength, without the elongation de-  
55 creasing. As the magnesium alloys of the kind

hitherto in use (electron, Dow-metal) have a  
comparatively small strength, this constitutes a  
further advance of considerable importance, the  
more so as the specific gravity of the alloys is  
scarcely increased to any perceptible extent by  
5 the small amount of the added metals.

Furthermore, the alloys according to the inven-  
tion show in comparison with similarly composed  
known electron alloys an increase of the perma-  
nent impact strength by 50%.

10 The alloys may be used as cast alloys or me-  
chanically worked alloys and may be improved  
by thermal treatments.

A satisfactory formula for an alloy according  
to my invention, in which aluminum and zinc  
15 are the principal additional ingredients, is as  
follows, viz:—

Magnesium 96.5%, aluminum 2%, zinc 1%, anti-  
mony 0.5%,

Magnesium 95.7%, aluminum 3%, zinc 1%, anti-  
mony 0.3%,

Magnesium 94.5%, aluminum 4%, zinc 1%, anti-  
mony 0.5%,

Magnesium 91.5%, aluminum 5%, zinc 3%, bis-  
muth 0.5%.

20 What I claim is:—

1. A low specific gravity magnesium base alloy  
containing from 80 to 97.8 per cent of magnesium,  
from 1.1 to 17 per cent of aluminum, from 1  
20 to 8.4 per cent of zinc, the content of aluminum  
exceeding that of zinc and the combined amount  
of aluminum and zinc being not more than 18  
per cent, from 0.05 to 2 per cent of a metal se-  
lected from the group consisting of antimony,  
30 35 and bismuth, the alloy being more resistant to  
corrosion than an alloy of the same composition  
but not containing a metal selected from the said  
group.

2. A low specific gravity magnesium base al-  
loy consisting of from 80 to 97.9 per cent of  
magnesium, from 1 to 17 per cent of aluminum,  
from 1 to 17 per cent of zinc, the combined  
35 content of aluminum and zinc being not more  
than 18 per cent, antimony more than 0.05 per  
cent, and bismuth more than 0.05 per cent, the  
sum of the contents of antimony and bismuth be-  
ing not more than 2 per cent.

40 3. A low specific gravity magnesium base al-  
loy consisting of from 80 to 97.95 per cent of  
magnesium, from 1 to 17 per cent of aluminum,  
from 1 to 17 per cent of zinc, the combined con-  
tent of aluminum and zinc being not more than  
45 50 55 18 per cent, and from 0.05 to 2 per cent of a

55

metal selected from the group consisting of antimony and bismuth.

4. As a new article of manufacture, an article resistant to corrosion and formed from an alloy containing magnesium, aluminum and zinc, the magnesium being present in an amount of from 80 to 97.8 per cent, the aluminum being present in an amount from 1.1 to 17 per cent, and the zinc from 1 to 8.4 per cent, the content of aluminum exceeding that of zinc and the combined amount of aluminum and zinc being not more than 18 per cent, and the alloy containing from 0.05 to 2 per cent of a metal selected from the group consisting of antimony and bismuth, the alloy being more resistant to corrosion than an alloy of the same composition but

not containing a metal selected from the said group.

5. A low specific gravity magnesium base alloy containing from 80 to 97.9 per cent of magnesium, from 1 to 17 per cent of aluminum, from 1 to 17 per cent of zinc, the combined amount of aluminum and zinc being not more than 18 per cent, antimony more than 0.05 per cent, and bismuth more than 0.05 per cent, the sum of the contents of antimony and bismuth being not more than 2 per cent, the alloy being more resistant to corrosion than an alloy of the same composition but not containing said antimony and bismuth.

GEORG SCHICHTEL. 1